

April 5, 1932.

R. R. SMITH ET AL

1,852,271

PROCESS OF ROLLING SHEETS

Original Filed Oct. 4, 1929



Russell R. Smith, William J. Tonger, <sup>INVENTOR.</sup>  
BY Lawbert A. Salender  
C. E. Allen  
ATTORNEYS

## UNITED STATES PATENT OFFICE

RUSSELL R. SMITH, WILLIAM F. SONGER, AND LAMBERT A. SALENDER, OF ASHLAND, KENTUCKY, ASSIGNORS TO THE AMERICAN ROLLING MILL COMPANY, OF MIDDLE-TOWN, OHIO, A CORPORATION OF OHIO

## PROCESS OF ROLLING SHEETS

Continuation of application Serial No. 397,314, filed October 4, 1929. This application filed February 18, 1930. Serial No. 429,297.

Our invention relates to methods of rolling metal, particularly iron and steel, in order to produce flat sheets of substantial width and length and of a relatively thin gauge.

5 This application is a continuation of our application Serial No. 397,314, filed October 4, 1929.

In the production of sheet metal by the continuous process great economies are affected, but these economies are dependent for their fullest advantage upon production on a very large scale because of the expensiveness of the equipment employed. Also 10 such continuous processes are only carried on to best advantage where large batches of uniform size pieces are run through the series of mills employed.

Our process is directed to the production 20 of a varied product, and to the utilization of a rough plate which can be considerably larger and also thinner than the sheet bars used in the customary sheet mill.

One of the objects of our process is to finish 25 rough plate material to desired gauge without reheating. Another object is to do away with the roughing mill operation used in the customary sheet production processes.

It is readily possible with the use of a continuous, two high universal mill or a heavy, 30 two high reversing mill, to produce fairly wide thick pieces of flat metal without restrictions as to length. Such material when made for the manufacture of pipe is termed "skelp" and it can be produced today, in widths up 35 to around sixty inches without great difficulty. Were wider or thinner material to be produced on such mills, a much heavier and more expensive equipment would have to be provided, and furthermore, very careful control of active pass applied to the pieces in the concluding stands of the mill would have to be exercised. This is largely due to the fact that wide pieces of flat material exercise great expansive force tending to separate the rolls of a mill, and thus spring them considerably unless they are extremely heavy, and to the further fact that when the metal is thin in gauge, it cannot flow laterally in the mill passes, and further, cannot be confined at the edges by means of mechanical

guides. Without very careful control of the active passes in the rolls, wide, thin material will therefore tend to elongate differently along one zone than along another, and will buckle or travel in a curve and run into the 55 necks of the mill rolls.

Our process utilizes with great economy, a rough product which is produced on mills, such as skelp mills or plate mills, where the difficulties last noted are not encountered, where the equipment is not relatively expensive, and the care in rolling is not nearly so paramount in importance. Heretofore the material used for rolling sheets has been called "sheet bar". Sheet bars are too narrow to 60 serve in our process, but if they are roughed down sufficiently to form proper pack forming material, we can finish such a pack in 65 our process without a reheating.

Ordinarily, the product which we employ in our process is the cheaply rolled plate material, which material is cut into lengths which 70 will correspond with the width of the final product, the pieces being rolled to a thickness which will give the desired length in the final product when reduced to the required gauge. We may also roll the plate sections lengthwise 75 of the preceding rolling step. We can also employ rough plate produced in fairly thick gauges on the modern continuous process 80 mills, which can furnish this material with great economy.

It should be noted that in order to provide an economical process of producing sheets, rolling equipment is called for which will 85 finish the rough product rapidly enough to warrant the use of a continuous furnace to supply the material in proper heated condition for rolling, and which will dispense with the intermediate reheating of the product 90 during the finishing.

This is provided for in our process by the use of a three-high mill, through which the pieces are passed to and fro, being rolled 95 first in one direction and then in the other. We preferably employ a tilting table at one side of the mill to catch the pieces as they are rolled, and lift them into the return pass, and heat the starting material in a continuous furnace at the entering side of the mill. 100

It would be impractical in any three-high mill, such as has been employed in the past in rolling plate, to finish the lighter gauges by our process, although three-high mills of the usual proportions may be used for the heavier gauges. This is because when the pieces come to the three-high mill in our process they are wide and very rapidly reduced to become quite thin, with corresponding rapid cooling, and maximum reductions per pass call for more rigid proportions combined with much smaller middle rolls than are ordinarily used in three-high mills. The proportions of the mills used in our process more closely resemble the modern continuous mills, which, however, are four-high mills.

In our process we provide for a three-high mill with a central roll of small diameter, and backing up rolls of considerably larger diameter which will result not only in a mill which is quite rigid as to its resistance to springing, but which permits the greater reduction of the pieces per pass than is possible with large diameter rolls engaging the piece. It is further advisable in our process to use very heavy housings in which the rolls are mounted, and to provide against elasticity in the roll supports, so that heavy drafts can be imparted. Furthermore, we preferably keep the rolls of the mill cold with water sprays.

So far as we are advised, it has never been proposed to roll packs or multiples of flat pieces in a three-high mill for one reason, because no mills have been designed for such a purpose, and because the process requires the use of wide plate material as distinguished from narrow bars for reduction to sheets without reheating, which has not occurred to those skilled in the art. In our process we reduce flat metal in multiples in the three-high mill, and effect great economies thereby.

As a guide in connection with the structure of the three-high mill, we have carried on our process in a mill with closed type housings, having a middle roll of a length of forty-eight to ninety-six inches, and a thickness of working barrel of fifteen inches, together with backing up rolls of like length of barrel, but with a thickness of thirty inches. In this mill the lower roll is driven, and the middle or small roll is idle. We do not confine our invention to the use of a mill of this one size, but believe that the thickness of the rolls proportionate to length is most desirable in a mill of the width used by us.

We have indicated in the appended drawings a diagram of a suitable mill arrangement to be used in our process.

In the drawings:—

Figure 1 is a diagram or plan of the mill.

Figure 2 is a vertical cross-section taken through the three-high mill.

The furnace 1, which is preferably a con-

tinuous furnace, delivers single thickness pieces to the table 2. The mill has the small central roll 3, and the outer rolls 4, 4, which are large in comparison to the roll 3. The table 5 is mounted so as to rock on the trunnions at 6. A water spray 7 is also provided.

In carrying out our process the pieces, which may be rough plate or bar of a wide range of width, thickness and length, is fed to the three-high mill from a continuous furnace. The pieces are passed through the mill between the middle and lower roll, and then back between the middle and upper roll until reduced to a length suitable for matching, whereupon the two pieces are matched, and the rolling continued in the same manner.

Instead of starting with rough plate or thin bar produced in a continuous mill or by continuous process, we may start with rough plate produced in any desired way.

Furthermore, referring now to the product of the modern continuous process mills, wherein the active pass is accurately controlled and large, heavy equipment provided, we can start our process with pairs which have not been given any treatment but a heating treatment, after leaving the continuous mill, if they are of thin enough gauge to permit this. The reason why we can do this is because the pieces rolled in such a process have a very definite shape given to them and the shape of the pairs furnished to the three-high mill, as in our process, can readily be determined.

Furthermore, we can start our process with a pair or pack which has been formed of pieces passed through a two-high roughing mill of usual type, provided care is taken in the roughing mill to produce pieces to be matched which have a definite contour.

In our process, once the individual pieces or packs have been started into the three-high mill, no reheating is given to the pieces, and they are rolled back and forth until they have been sufficiently reduced. In producing finer gauges three rough plates may be started through the mill, the catcher holding one and passing one for the first few passes, and then matching all three, and finishing the pieces as a pack of three.

In one typical process the individual pieces from a skelp mill of .2 inches thickness are fed through once by the roller, and back once by the catcher, whereupon the roller matches them, and three more passes are given to the pair, giving a product of .062 inches or 16 gauge. We find that mechanically operated tilting and catching tables are of advantage in gaining fullest benefit from our process.

In another typical process, pieces from the modern continuous mills, having a thickness of .085 inches, can be rolled down in three to five passes, depending upon the

number of elements of the pack, without any introductory individual passage of the elements through the mill, to a gauge of .035 to .031 for the resulting product.

5 Also, ordinary sheet bars may be passed through a roughing mill and reduced to proper gauge, say .140 inches, for forming a pair, and this pair then passed to and fro in the three-high mill without any reheating 10 to a finished thickness of .05 inches or 18 gauge.

These, of course, are merely given as examples of what may be done with our process, as thicker or thinner packs or pieces may 15 be used to start with than in any of the examples, and thinner or thicker gauges of final product formed. The limitations in final gauge depend upon the necessity for reheating if the pieces get too cold, the thickness 20 of the starting material and number of pieces in the pack, two being the best number in our experience.

We believe that it is a necessary feature 25 of our process to finish to final gauge as a pair, or in multiple without doubling, which of itself is novel in sheet mill practice except for certain continuous processes of sheet rolling to which we have referred. If doubling were attempted, the time lost would 30 require a reheating, which would cause loss of time and great expense.

By using a three-high mill of great rigidity and heavy draft, using it to reduce the starting material by passes in single thickness, or using a roughing mill to form a pair which itself is rapid and economical, and then finishing in two thicknesses in the three-high mill, we have been able to take the product from a continuous furnace, operating 35 on an economical basis and very greatly reduce the cost of producing sheet metal over the hand mill rolling art. Indeed, for anything but a very large production, the results of using our process have 40 been more economical than any process of sheet rolling known at the present time, including the continuous mill production, and continuous process, tandem rolling.

The use of the water cooling of the three-high mill of our invention is of importance 50 in a number of respects. The mill, of course, must have the small diameter middle roll and thus we are permitted to gain great reductions in each pass without excessive pressure, 55 and the rigidity of the mill inhibits great springing of the rolls. In spite of this, however, the presence of a film of water on the rolls, thus keeping them cold, makes our process much more practical.

60 The shape of the rolls is easier to control because there is little or no variation due to differential heating of the rolls. Due to the fact that the pores of the metal in the rolls are kept closed because of the low temperature thereof during rolling, the sur-

face of the rolls are not subjected to marking, and the flow of water over the rolls tends to remove tiny particles of grit, in the short idle time between passes. It is practical to use higher initial temperature of the 70 pieces with the water cooled three-high mill, because with water cooled rolls, effecting desired reductions per pass with a minimum of applied pressure, the tendency of the parts of a pack to become stuck together or to 75 "patch" and stick due to partial welding of the surfaces is largely done away with. This last seems to be due to the fact that setting and patching are the results of combined pressure and temperature, setting taking 80 place when both are high, and patching when both are low, and that with the water cooled three-high mill with small diameter working roll, the combination of pressure and temperature will not result in patching or sticking. 85

The advantage in accuracy of production of the process of our invention will be evident from the fact that we can finish a pack on our three-high mill, and then reheat it and 90 roll it in doubled or re-matched shape on an ordinary two-high hot hand mill, without difficulty.

We do not know of any process in the past 95 whereby packs of substantial width can be rolled by repeated passes on one mill, and then reheated, doubled or matched to greater thickness, and successfully finished on another mill on a commercial basis to light gauges. This is possible in our process, because the water cooled three-high mill operating as it does, produces packs of a very accurate contour, and the finishing roller can arrange a proper setting for his finishing mill to take care of the initial passes of the 100 packs furnished to him, and "set" the pack so that it can be rolled tight.

As compared to the customary process of 105 finishing sheets in pairs and packs, the difference of our process is apparent.

As compared to process in which the three-high mill has been employed in rolling plates, using a tilting catching table, and reducing in the reverse as well as the forward pass, the structure of mill as to rigidity, comparative size of inner and outer rolls, and lack of springiness in the mill during the active pass, permits us to use large sized rough plate, and roll in multiple or first singly and then in multiple to finished gauge without reheating 110 material. Furthermore, since we reduce, first singly and then in pairs or multiple, we produce a very much finer gauge material than was ever produced on the to and fro rolling in three-high plate mills of the past; in which single thickness has invariably been produced. Indeed, we start our process with material which is comparable in thickness to about the finest gauge that was ever finished commercially on the three-high plate mill. 115

Having thus described our invention, what we claim as new and desire to secure by Letters Patent, is:—

1. In a process of rolling sheets, the steps of passing heated pieces longer in direction of rolling than ordinary sheet bars singly, first between a small central roll and large bottom roll, and then back between the small central roll and a large top roll, sufficiently to reduce the pieces to pack forming material, then matching the single pieces into a pack and without reheating, continuing to pass the pack forth and back in the same manner between the same rolls, the rolls so employed being kept cold enough to substantially eliminate change of shape due to heating.

2. In a process of rolling sheets, the steps of passing heated sections of continuously rolled plates longer in direction of rolling than ordinary sheet bars singly, first between a small central roll and large bottom roll, and then back between the small central roll and a large top roll, sufficiently to reduce the pieces to pack forming material, then matching the single pieces into a pack and without reheating, continuing to pass the pack forth and back in the same manner between the same rolls.

3. In a process of rolling sheets, the steps of passing heated pieces longer in direction of rolling than ordinary sheet bars singly, first between a small central roll and large bottom roll, and then back between the small central roll and a large top roll, sufficiently to reduce the pieces to pack forming material, then matching the single pieces into a pack and without reheating, continuing to pass the pack forth and back in the same manner between the same rolls, said pieces being furnished to the first pass from a continuous furnace.

4. In a process of rolling sheets that step which consists in rolling a pack of heated flat material longer in direction of rolling than ordinary sheet bars, first between a small central roll and large bottom roll, and then back between the small central roll and a large top roll, and continuing in this sequence without doubling to desired gauge, the rolls so employed being kept cold enough to substantially eliminate change of shape due to heating.

5. In a process of rolling sheets that step which consists in rolling a pack of heated flat material, first between a small central roll and large bottom roll, and then back between the small central roll and large top roll, and continuing in this sequence without doubling to finished gauge, the pack being formed of material given at least one pass between said rolls previous to being matched.

6. In a process of rolling sheets, the steps of passing heated pieces longer in direction of rolling than an ordinary sheet bar singly,

first between a small central roll and large bottom roll, and then back between the small central roll and a large top roll, sufficiently to reduce the pieces to pack forming material, then matching the single pieces into a pack and without reheating, continuing to pass the pack forth and back in the same manner between the same rolls, the said rolls being kept cold by water during the process, sufficiently to eliminate substantial change of shape due to heating and to maintain the roll surface and avoid setting and patching.

7. In a process of rolling sheets, the steps of passing heated pieces singly, first between a small central roll and large bottom roll, and then back between the small central roll and a large top roll, sufficiently to reduce the pieces to pack forming material, then matching the single pieces into a pack and without reheating, continuing to pass the pack forth and back in the same manner between the same rolls, the said rolls being kept covered with a film of water during the process, the said pieces furnished at the start of the process being longer in the direction of rolling than a sheet bar.

8. In a process of rolling sheets that step which consists in rolling a pack of flat material, first between a small central roll and large bottom roll, and then back between the small central roll and a large top roll, and continuing in this sequence without doubling to desired gauge, the rolls being kept covered with a film of water during the process.

9. In a process of rolling sheets that step which consists in rolling a pack of flat material, first between a small central roll and large bottom roll, and then back between the small central roll and a large top roll, and continuing in this sequence without doubling to desired gauge, the rolls being kept covered by a film of water during the process so as to eliminate substantial change of shape thereof due to heating, and then doubling or matching and reheating the packs and rolling same on a finishing mill.

RUSSELL R. SMITH.  
WILLIAM F. SONGER.  
LAMBERT A. SALENDER.

115

120

125

130

70

75

80

85

90

95

100

105

110

115